

[54] LIGHT-SENSITIVE SUPER-SENSITIZED SILVER HALIDE PHOTOGRAPHIC EMULSION

[75] Inventors: **Shui Sato**, Tokyo; **Eiichi Sakamoto**, Hanno; **Yuji Watanabe**, Saitama-ken; **Kaichiro Sakazume**; **Tokuo Kaneko**, both of Tokyo, all of Japan

[73] Assignee: **Konishiroku Photo Industry Co., Ltd.**, Tokyo, Japan

[22] Filed: **July 11, 1972**

[21] Appl. No.: **270,830**

**Related U.S. Application Data**

[63] Continuation-in-part of Ser. No. 18,622, March 11, 1970, abandoned.

[30] **Foreign Application Priority Data**

Mar. 14, 1969 Japan..... 44/18898

[52] U.S. Cl..... 96/124, 96/100

[51] Int. Cl..... G03c 1/14

[58] Field of Search..... 96/124, 137

[56] **References Cited**

UNITED STATES PATENTS

|           |        |                  |        |
|-----------|--------|------------------|--------|
| 3,663,210 | 5/1972 | Sato et al.....  | 96/124 |
| 3,666,480 | 5/1972 | Shiba et al..... | 96/124 |
| 3,713,835 | 1/1973 | Sato et al.....  | 96/124 |
| 3,718,475 | 2/1973 | Shiba et al..... | 96/124 |

Primary Examiner—J. Travis Brown

Attorney—Eric H. Waters et al.

[57] **ABSTRACT**

A green-sensitive supersensitizer for light-sensitive sil-

ver halide photographic emulsions comprises a combination of at least one dye represented by the formula:



wherein  $\text{R}_1$  is a lower alkyl group,  $\text{R}_2$  is a sulfoalkyl group, a carboxyalkyl group or a derivative of any of said groups,  $\text{W}_1$  and  $\text{W}_2$  are individually a hydrogen atom or a lower alkyl group,  $\text{Z}$  is a sulfur or selenium atom,  $\text{X}^-$  is a negative group, and  $n$  is 1 or 2 and at least one dye represented by the formula:



wherein  $\text{R}_3$  and  $\text{R}_4$  are individually a lower alkyl group or a substituted alkyl group,  $\text{R}_5$  and  $\text{R}_6$  are individually a lower alkyl group, a hydroxyalkyl group, a sulfoalkyl group or a derivative of any of said groups,  $\text{Y}_1$  and  $\text{Y}_2$  are individually a n-propyl, iso-propyl, n-butyl, iso-butyl or phenyl group,  $\text{X}^-$  is a negative group, and  $n$  is 1 or 2.

**3 Claims, No Drawings**

**LIGHT-SENSITIVE SUPER-SENSITIZED SILVER  
HALIDE PHOTOGRAPHIC EMULSION**

**CROSS REFERENCE TO RELATED  
APPLICATIONS**

5

This application is a continuation-in-part application of Ser. No. 18,622 filed Mar. 11, 1970, now abandoned.

This invention relates to a light-sensitive silver halide photographic emulsion containing a combination of spectral sensitizing dyes. More particularly, the invention is concerned with a green-sensitive supersensitizer comprising a monomethinecyanine dye and a benzimidazolocarbocyanine dye.

A silver halide photographic emulsion has an inherent light-sensitive wavelength region. This wavelength region, however, is ordinarily limited to the short wavelength region of ultraviolet light or blue light. When such silver halide emulsion is incorporated with a sensitizing dye, the emulsion is broadened in light-sensitive wavelength region and thus can be sensitized. Further, it is well known that when a mixture of a spectral sensitizing dye with other spectral sensitizing dye or with an organic compound is added to a silver halide emulsion, the emulsion is sensitized to more than the total sum of the effects of the individual compounds. This phenomenon is termed supersensitization, and is detailed in, for example, C.E.K. Mees: "The Theory of the Photographic Process," 2nd. Edition, 1954, New York, page 474.

When subjected to development treatment, a photographic film or paper prepared by use of a green-sensitive silver halide photographic emulsion containing a conventional supersensitizing composition has tended to bring about yellow color stain of magenta color. This tendency is particularly marked when the emulsion contains a gelatine coagulant.

Further, the use of a certain known supersensitizing composition gives a light sensitive material which, when stored at high temperature and high humidity, brings about a decrease of photographic gamma. This is ascribable to the fog formed in the emulsion layer during storage of the light-sensitive photographic material. Even if the proportions of the dyes in said supersensitizer are varied so as to prevent the decrease of photographic gamma, the light-sensitive photographic material is undesirably varied in sensitization maximum to bring about a decrease of green sensitivity.

An object of the present invention is to provide a supersensitizer having stable green-sensitivity even at high temperature and high humidity which has overcome the above-mentioned drawbacks of conventional supersensitizers and which does not bring about any dye contamination in the resulting film after treatment.

Another object of the invention is to provide a light-sensitive silver halide photographic emulsion having high green sensitivity (high speed to green light), which emulsion is less in generation of optical fog even when handled under a safety light having a wavelength of more than 600 m $\mu$ .

The above objects of the present invention are accomplished by the use of a combination of at least one of the monomethinecyanine dyes of the general formula (I) shown below and at least one of the benzimidazolocarbocyanine dyes of the general formula (II) also shown below. General formula (I):



wherein R<sub>1</sub> is a lower alkyl group, R<sub>2</sub> is a sulfoalkyl group, a carboxyalkyl group or a derivative of any of said groups, W<sub>1</sub> and W<sub>2</sub> are individually a hydrogen atom or a lower alkyl group, Z is a sulfur or selenium atom, X<sup>-</sup> is a negative group, and n is 1 or 2. General formula (II):

15



wherein R<sub>3</sub> and R<sub>4</sub> are individually a lower alkyl group or a substituted alkyl group, R<sub>5</sub> and R<sub>6</sub> are individually a lower alkyl group, a hydroxylalkyl group, a sulfoalkyl group or a derivative of any of said groups, Y<sub>1</sub> and Y<sub>2</sub> are individually a n-propyl, iso-propyl, n-butyl, iso-butyl or phenyl group, X<sup>-</sup> is a negative group, and n is 1 or 2.

All the spectral sensitizing dyes or the above-mentioned general formulas are ortho type spectral sensitizing dyes, and the sensitizing dyes of the general formula (I) are green-sensitizing dyes showing a maximum wavelength of color sensitization within a short wavelength region of 500 m $\mu$  to 550 m $\mu$ , while those of the general formula (II) are green-sensitizing dyes showing color sensitization maximum at a long wavelength region of 570 m $\mu$  to 580 m $\mu$ . When used singly, therefore, these sensitizing dyes cannot give green-sensitive silver halide photographic emulsions the color sensitivity of which has been sufficiently broadened in wavelength region.

As the result of extensive studies, we have found that when the spectral sensitizing dyes of the general formulas (I) and (II) are used in combination with each other, there is attained marked green-sensitization due to the synergistic effect of said spectral sensitizing dyes.

That is, when a combination of said two kinds of spectral sensitizing dyes is added to a silver halide photographic emulsion, the emulsion is sensitized in short wavelength portion and long wavelength portion of the green light-sensitive spectral zone, whereby there are attained not only high speed green-sensitivity but also green sensitization having a new spectral sensitization maximum which cannot be attained when these spectral sensitizing dyes are used singly. Further, the combination of the two spectral sensitizing dyes has such excellent characteristics that it has no detrimental interactions with other photographic additives and does not leave any residual color stain on a photographic film after development.

The sensitizing dyes of the general formula (I) are synthesized by use of quaternary 2-alkylmercaptoquinonium salts, and those of the general formula (II) are obtained according to the methods described in U.S. Pat. No. 3,268,334.

Typical examples of the spectral sensitizing dyes represented by the general formulas (I) and (II) are shown below, but it is needless to say that compounds usable in the present invention are not limited only to these. Typical examples of the spectral sensitizing dyes of the general formula (I):

(1)



(2)



(3)



(4)



10 (6)

15



20 (6)



25 Typical examples of the sensitizing dyes represented by the general formula (II):

(7)



(8)



(9)



(10)



(11)





The supersensitizers according to the present invention have such excellent characteristics as mentioned previously and can impart ideal green-sensitivity to silver halide photographic emulsions. Accordingly, the super-sensitizers of the present invention are highly effective as color sensitizers not only for green-sensitive emulsions for high speed, light-sensitive, black-and-white photographic materials but also for green-sensitive emulsions for light-sensitive color photographic materials.

The silver halide photographic emulsions in accordance with the present invention can be varied in distribution of spectral sensitization maximum wavelengths by varying the kind and amount of the spectral sensitizing dyes of the aforesaid general formulas. These sensitizing dyes may be added to silver halide photographic emulsions after dissolving them, either singly or in admixture, in a water miscible organic solvent such as methanol, ethanol or the like. Further, the spectral sensitizing dyes may be added to the emulsions at any time during preparation of the emulsions, but are preferably added immediately after completion of second ripen-

ing, in general. The amounts of the spectral sensitizing dyes to be added vary depending on the kind of silver halide emulsions, but are ordinarily within such a wide range that the total amount of the spectral sensitizing dyes of the formulas (I) and (II) is 1 mg. to 200 mg. per Kg. of the emulsion. In this case, the ratio of the dye of the formula (I) to that of the formula (II) is preferably within the range of 1:10 to 10:1 by weight.

The silver halide photographic emulsions usable in the present invention may be any of silver iodobromide, silver chlorobromide, silver bromide and silver chloride emulsions. These emulsions may have been sensitized with noble metal sensitizers, sulfur sensitizers, reduction sensitizers or polyalkylene oxide type sensitizers. Further, the emulsions may have been incorporated according to known procedures with such additives as stabilizers, surface active agents and hardeners.

In the above-mentioned color sensitization process of the present invention, other carbocyanine or merocyanine dyes may be additionally used to provide high speed spectral sensitivity, so that it is possible to carry

out easily spectral sensitization for light-sensitive black-and-white photographic materials using various silver halides.

The present invention is illustrated in further detail below with reference to examples.

### EXAMPLE 1

A silver iodobromide emulsion containing 3 mole percent of silver iodide which had been treated with a gelatine coagulant was subjected to second ripening following sensitization with gold and sulfur, thereby to prepare a neutral emulsion for high speed negatives. To 1 Kg. of this emulsion was added, either singly or in admixture in such amount as shown in Table 1, 0.1 percent methanol solutions of the spectral sensitizing dyes of the aforesaid general formulas (I) and (II). The emulsion was allowed to stand with stirring at about 40°C. for 20 minutes, the spectrally sensitized emulsion thus obtained was then coated on a film base, followed by drying, to obtain a green-sensitive photographic material. For the purpose of sensitometry, the thus obtained photographic material was exposed to light through a yellow light filter by means of a sensitometer KS-1 (manufactured and sold by Konishiroku Photo Industry Co., Ltd.) at 100 Lux and at 5,400°K., developed at 20°C. for 5 minutes with a developing solution of the composition shown below, and subjected to fixing, water-washing and drying.

Developing solution:

|                                        |          |
|----------------------------------------|----------|
| Metol (N-methyl-p-aminophenol sulfate) | 3 g.     |
| Anhydrous sodium sulfite               | 50 g.    |
| Hydroquinone                           | 6 g.     |
| Sodium carbonate (monohydrate)         | 29.5 g.  |
| Potassium bromide                      | 1 g.     |
| Water to make                          | 2 liters |

Further, the spectral sensitivity was measured by exposing each sample by use of a gating spectrograph and then developing the exposed sample. The results obtained were as set forth in Table 1. In the table, the sensitivity value is represented by a relative value, regarding as 100 the yellow sensitivity of a film sensitized by adding, per Kg. of the emulsion, 60 mg. of the sensitizing dye of the general formula (I). The residual color stain is a density measured by means of a color densitometer.

TABLE 1

| Sample No. | Spectral sensitizing dye<br>Exemplification No. | General formula | Amount added<br>(0.1% cc./<br>kg. emulsion) | Relative speed to<br>yellow light | Residual color stain | Spectral sensitivity maximum<br>( $\mu$ ) |
|------------|-------------------------------------------------|-----------------|---------------------------------------------|-----------------------------------|----------------------|-------------------------------------------|
| 1          | (1)                                             | [I]             | 60                                          | 100                               | 0.06                 | -----                                     |
| 2          | (8)                                             | [II]            | 60                                          | 170                               | 0.07                 | -----                                     |
| 3          | (1)+(8)                                         | [I]+[II]        | 40+20                                       | 210                               | 0.04                 | 570                                       |
| 4          | (6)                                             | [I]             | 50                                          | 95                                | 0.07                 | -----                                     |
| 5          | (13)                                            | [II]            | 60                                          | 160                               | 0.06                 | -----                                     |
| 6          | (6)+(13)                                        | [I]+[II]        | 35+25                                       | 205                               | 0.04                 | 575                                       |
| 7          | (3)                                             | [I]             | 60                                          | 80                                | 0.06                 | -----                                     |
| 8          | (9)                                             | [II]            | 60                                          | 150                               | 0.06                 | -----                                     |
| 9          | (3)+(9)                                         | [I]+[II]        | 40+20                                       | 190                               | 0.03                 | 570                                       |

From the above table, it is understood that the Samples 3, 6 and 9 in accordance with the present invention have markedly enhanced, as compared with other samples, the spectral sensitivity of the resulting photographic materials, and that even when added to emulsions prepared by use of a gelatine coagulant, they do

not injure the photographic properties thereof and make the emulsions less in color stain (residual color) on the films after development.

The accompanying drawings FIGS. 1 and 2 are spectral sensitivity curves. In FIG. 1, the curve (a) shows the spectral sensitivity curve of a photographic material using the silver iodobromide emulsion prepared in Example 1, and the curves (b) and (c) show, respectively, the spectral sensitivity curves of the Samples 1 and 2 obtained in Example 1. In FIG. 2, the curve (d) shows the spectral sensitivity curve of the Sample 3 obtained in Example 1. From these drawings also, it is understood that the photographic emulsions according to the present invention have excellent photographic properties.

### EXAMPLE 2

To 1 Kg. of a high speed silver iodobromide emulsion prepared according to an ordinary process were added, in such combinations and amounts as shown in Table 2, spectral sensitizing dyes of the general formulas (I) and (II).

After spectral sensitization, each of the emulsions was incorporated with a suitable amount of 4-hydroxy-6-methyl-1,3,3a,7-tetraazaindene as an antifogant and then coated on a film base, followed by drying, to obtain a green-sensitive photographic material. On the other hand, a combination of the control dye (A) and the control dye (B) shown below, which combination is disclosed in U.S. Pat. No. 2,701,198, was treated in the same manner as above to obtain a control sample. Control dyes:

(A)



(B)



Each of the thus obtained samples was subjected to storage test at high temperature and high humidity to obtain such results as shown in Table 2.

The exposure, development and sensitometry in this example were effected in the same manner as in Example 1, and the sensitivity value in the table was represented by a relative sensitivity based on that of the control sample.

TABLE 2

| Sample No. | Sensitizing dye      | Amount added<br>(cc./kg.<br>emulsion) | Immediately after preparation        |       |      | After incubation for 3 days<br>at 50° C., RH 80% |       |      |
|------------|----------------------|---------------------------------------|--------------------------------------|-------|------|--------------------------------------------------|-------|------|
|            |                      |                                       | Relative<br>speed to<br>yellow light | Gamma | Fog  | Relative<br>speed to<br>yellow light             | Gamma | Fog  |
| 10         | (2) plus (8)         | 40+20                                 | 130                                  | 0.74  | 0.04 | 130                                              | 0.72  | 0.05 |
| 11         | (2) plus (14)        | 35+25                                 | 110                                  | 0.71  | 0.04 | 115                                              | 0.73  | 0.05 |
| 12         | (3) plus (8)         | 40+20                                 | 125                                  | 0.73  | 0.06 | 125                                              | 0.72  | 0.06 |
| 13         | (3) plus (14)        | 30+30                                 | 120                                  | 0.70  | 0.05 | 110                                              | 0.70  | 0.05 |
| 14         | Control (A) plus (B) | 40+20                                 | 100                                  | 0.72  | 0.07 | 95                                               | 0.65  | 0.08 |

From Table 2, it is evident that even when stored under severe conditions, the light-sensitive materials 10, 11, 12 and 13 according to the present invention are less in formation of fog and can display excellent photographic properties without degradation of photographic sensitivity and gamma.

**EXAMPLE 3**

A high speed silver iodobromide emulsion, which had been second ripened to the optimum sensitivity after gold and sulfur sensitization, was divided into 3 portions. To 1 Kg. of each divided portion of the emulsion were added, in such combinations as shown in Table 3, the spectral sensitizing dyes of the aforesaid general formulas (I) and (II). For comparison, the same control sample as in Example 2 was used. Each of the thus treated emulsions was allowed to stand with stirring at 40°C. for about 20 minutes. Thereafter, the thus spectrally sensitized emulsion was charged with a hardener and a coating aid and then coated on a film base, followed by drying, to prepare a sample.

In order to test each of the thus prepared samples in optical fog formation under red light, the sample was continuously irradiated, through a filter (Sakura No. 4-A) capable of transmitting a light of more than 600 m $\mu$  in wavelength, with a light positioned at a distance of 100 cm. from the sample (the light source used was an incandescent lamp of 100V-20W).

After irradiation, the samples were developed in the same manner as in Example 1 and then measured in fog density to obtain the results as shown in Table 3.

The results of sensitometry effected in the same manner as in Example 1 were also set forth in Table 3.

From Table 3, it is understood that the light-sensitive photographic emulsions of the present invention are advantageously less in optical fog formation under red light.

## 15 Experiment 4

Experiment 4  
A silver iodobromide emulsion containing 3 mole percent of silver iodide which had been treated with a gelatine coagulant was subjected to second ripening following sensitization with gold and sulfur, thereby to prepare a neutral emulsion for high speed negative. To 1 Kg. of this emulsion was added, either singly or in admixture in such amount as indicated in Table 1 below, 0.1 percent methanol solutions of the sensitizing dyes represented by the general formulas (I) and (II) of the present specification. For comparison, a compound set forth in claim 10 of U.S. Pat. No. 3,268,334 was similarly used to prepare a control sample.

The emulsions were allowed to stand with stirring at about 40°C. for 20 minutes to complete colour sensitization. The sensitized emulsions were then coated on a film base and dried to prepare green-sensitive photographic materials. The sensitive photographic materials were exposed through a yellow light filter in accordance with the method JIS 1604-K, developed at 20°C. for 5 minutes with a developing solution described in the specification, fixed, washed with water, dried and subjected to sensitometry. The results obtained were shown in Table 1 below. In the table, the sensitivity value is represented by a relative value, rating as 100 the yellow sensitivity of a photographic film added with the following sensitizing dye (1) according to the present invention in the amount of 60 mg. per Kg. of the emulsion. The residual color stain is a density measured

5 by means of a color densitometer.  
Thus, according to the present inventi-

TABLE 2

| Sample No. | Sensitizing dyes     | Amount added<br>(0.1%<br>cc./kg.<br>emulsion) | Red light irradiation time |         |         | Relative speed to<br>yellow light |
|------------|----------------------|-----------------------------------------------|----------------------------|---------|---------|-----------------------------------|
|            |                      |                                               | 0 min.                     | 10 min. | 20 min. |                                   |
| 15.        | (5) plus (8)         | 30+20                                         | 0.05                       | 0.06    | 0.08    | 130                               |
| 16.        | (5) plus (14)        | 30+20                                         | 0.06                       | 0.07    | 0.09    | 115                               |
| 17.        | (1) plus (13)        | 30+20                                         | 0.05                       | 0.06    | 0.07    | 120                               |
| 18.        | Control (A) plus (B) | 30+20                                         | 0.05                       | 0.10    | 0.15    | 100                               |



For Comparison (U.S. Pat. No. 3,268,334)  
Control dye (Example 9 of U.S. Pat. No. 3,268,334)



wherein R<sub>3</sub> and R<sub>4</sub> are individually a lower alkyl group, a hydroxyalkoxyalkyl group or methoxycarbonylalkoxyalkyl group, R<sub>5</sub> and R<sub>6</sub> are individually a lower alkyl group, a hydroxyalkyl group or a sulfoalkyl group, Y<sub>1</sub> and Y<sub>2</sub> are individually a n-propyl, iso-propyl, n-butyl, iso-butyl or phenyl group, X<sup>-</sup> is a negative group, and n is 1 or 2.

2. A light-sensitive silver halide photographic emulsion as claimed in claim 1, said emulsion being a color photographic emulsion.

5 3. A light-sensitive silver halide photographic emulsion as claimed in claim 1, further comprising at least one magenta coupler.

\* \* \* \* \*